

Feb. 3, 1953

C. W. STRATFORD

2,627,496

PROCESS FOR WASHING ACID TREATED DISTILLATE

Filed Feb. 25, 1950

2 SHEETS—SHEET 1



Fig. 1.

INVENTOR.  
Charles Walcott Stratford  
BY *John E. Scoville*  
ATTORNEY.

Feb. 3, 1953

C. W. STRATFORD

2,627,496

PROCESS FOR WASHING ACID TREATED DISTILLATE

Filed Feb. 25, 1950

2 SHEETS--SHEET 2



Fig. 2.

INVENTOR,  
Charles Walcott Stratford

BY *Thos. E. Scoglied*  
ATTORNEY.

## UNITED STATES PATENT OFFICE

2,627,496

PROCESS FOR WASHING ACID TREATED  
DISTILLATECharles Walcott Stratford, Kansas City, Mo., as-  
signor to Stratford Engineering Corporation,  
Kansas City, Mo., a corporation of Delaware

Application February 25, 1950, Serial No. 146,378

3 Claims. (Cl. 196—41)

1

This invention relates to improvements in a process for washing acid treated distillates and refers more particularly to a process for removing salts of sulfonic bodies, ash or color-bearing constituents from lubricating oil distillates previously treated with acid.

The process is an improvement over that described in Patent 1,927,853 and an application Serial No. 95,702 filed May 27, 1949, now Patent No. 2,585,874. As described in these prior cases, the washing of the oil was conducted by water washing the distillate in one or more stages to remove objectionable constituents. With some oils purification sufficient to meet specification requirements cannot be obtained by simple water washing methods. The use of steam, however, readily brings the oil, after acid treating and neutralization, to the desired specifications with little difficulty.

An object of the invention, therefore, is to provide a method of washing lubricating oil distillates, which have been acid treated, with steam to remove ash, color bearing constituents and salts of sulfonic bodies.

Another object is to prevent loss of color of the oil which takes place in water washing methods heretofore used reducing the amount of acid dosage required to produce a specified color.

A further object is to eliminate emulsions frequently formed by conventional water washing and make the gravity separation of the oil from the washing fluids more rapid and complete.

Other objects and advantages will be apparent from the description which follows.

In the accompanying drawings which form a part of the specification and are to be read in conjunction therewith and in which like reference numerals indicate like parts in the various views,

Fig. 1 is a schematic flow diagram of a portion of a treating system embodying the invention.

Fig. 2 is a graph in which NPA color is charged against acid dosage pounds per barrel of charge.

In Fig. 1 of the drawings there is shown only that portion of the system which has to do with the neutralizing and finishing of the oil undergoing treatment. The sour oil from the acid treatment which precedes arrives through pipe 10 and is passed through heat exchanger 11 to increase or decrease its temperature within a satisfactory range for the neutralization treatment which follows. A heating or cooling medium is supplied to the exchanger through pipe 12 and the temperature of this medium is regulated by the outlet temperature of the oil discharged from

2

the exchanger through pipe 13. To accomplish this regulation, connections of the control device 14 are interposed in the discharge line 13 and operate valve 15 which regulates the amount of cooling or heating medium supplied to the exchanger. After being heated to the proper degree the oil is charged to a motor driven contacting device 16 where it is intimately mixed with a neutralizer supplied to the contactor through pipe 17. In this stage the sour oil and alkali are combined at relatively elevated temperatures and under sufficient pressure to keep all components of the mixture in liquid phase after which the mixture is passed to heat exchanger 18. The temperature within this exchanger is similarly controlled as in exchanger 11 by a temperature control device 14. From heat exchanger 18 the oil and alkali mixture is passed through pipe 20 to a settler 21 where separation of the neutralizer from the oil is effected. The neutralizer is passed to drum 22 and the oil is removed through pipe 23 through which it is directed to a steam mixer 24. Neutralizer collected in the drum 22 is recycled through pipe 25 and by means of pump 26 is recirculated to the neutralizing contactor 16 through pipe 17. A withdrawal line 27 controlled by valve 28 may be used to remove spent soda or other neutralizer from the system from time to time as desired. Fresh neutralizer is mixed in make-up tank 29 and is supplied to the system through pipe 30.

In some instances it may be necessary to carry a higher temperature in the neutralizing settler 21 than is employed in the preceding contacting step 16 for purposes of facilitating the gravity separation of the alkali solution from the oil. It is for this reason that the heat exchanger 18 is provided before the mixture enters the settler. Pressure on the settler is held sufficiently high to prevent vaporization of water or oil. When neutralization is accomplished under conditions of elevated temperature and pressure the optimum strength of the neutralizing system in the case of caustic soda solution may vary between 2% and 30% on the dry base caustic soda.

In the first stage steam wash mixer 24, steam is supplied through pipe 31 to be mixed with the oil for the purpose of removing alkali salts of sulfonic bodies or color-bearing constituents. The effluent flows through pipe 32 into heat exchanger 33 likewise regulated by temperature control device 14, as were the previous heat exchangers in the system. The temperature to which the oil-steam mixture is cooled in this heat exchanger must be such as

required to insure complete condensation of the steam but as little below that temperature as practical to maintain, so that the condensed steam will readily settle in condensate settler 34 to which the oil is passed through pipe 35. The wash condensate water is drawn off continuously from the bottom of the settler through pipe 36, while the oil is removed from the top through pipe 37. It is contemplated that one or more steam washing stages may be required and in the drawings there has been shown a two-stage system. The second stage steam wash mixer is diagrammatically shown at 38 to which the oil is supplied through pipe 37 and steam is introduced to the second stage mixer through pipe 38a. From the second steam washing stage the oil and steam are passed through pipe 38b through heat exchanger 39 regu-

stage water washing operations, one in which the acid dosage corresponded to that employed in the steam washing operation and the other with an acid dosage that produces a final NPA color corresponding to the steam washed treat, the treating conditions, amounts of steam and water employed for the washing operations; an analysis of the product from the different operations and a brief survey showing the ash removal per washing stage as well as the percentage yield of finished oil. The process is particularly adapted to relatively heavy oils above 500 viscosity SSU at 100° F. The oil treated in the operations included within the tabulation was a distillate having a viscosity of approximately 2200 Saybolt Seconds Universal at 100° F. originating from a naphthenic base Texas Coastal crude oil.

| Treating Conditions            | Charge Stock | 3-Stage Steam Injection Washing | Charge Stock | 3-Stage Water Washing | Charge Stock | 3-Stage Water Washing |
|--------------------------------|--------------|---------------------------------|--------------|-----------------------|--------------|-----------------------|
| Acid Dosage, #/bbl. oil        | 0.0          | 6.0                             | 0.0          | 6.0                   | 0.0          | 16.5                  |
| Acid Treating, Temp., ° F.     |              | 175                             |              | 175                   |              | 175                   |
| Total Steam, #/bbl. Oil        | None         | 365                             | None         | None                  | None         | None                  |
| Total Water, #/bbl. Oil        | None         | None                            | 4,200        | None                  | None         | 4,200                 |
| Product Inspection:            |              |                                 |              |                       |              |                       |
| Gravity, ° A. P. O.            | 21.0         | 20.9                            | 20.4         | 21.0                  | 20.5         | 21.3                  |
| Viscosity, SUV, at 100° F.     | 2,219        | 2,064                           | 2,082        | 1,866                 | 2,184        | 1,853                 |
| Viscosity, SUV, at 210° F.     | 98.6         | 96.4                            | 95.4         | 92.6                  | 98.0         | 92.6                  |
| Color, NPA                     | 8+           | 4½                              | 8+           | 6                     | 8+           | 4½                    |
| Carbon Residue                 | 0.24         | 0.33                            | 0.46         | 0.55                  | 0.44         | 0.53                  |
| Neutralization No.             | 0.04         | 0.03                            | 0.03         | 0.04                  | 0.06         | 0.04                  |
| Ash percent                    | Nil          | Nil                             | Nil          | 0.04                  | Nil          | .058                  |
| Ash Removal Per Washing Stage: |              |                                 |              |                       |              |                       |
| Caustic Washed Oil             |              | 0.450                           |              | 0.450                 |              | 0.550                 |
| 1st Stage Ash, percent         |              | 0.111                           |              | 0.140                 |              | 0.190                 |
| 2nd Stage Ash, Percent         |              | 0.003                           |              | 0.084                 |              | 0.068                 |
| 3rd Stage Ash, Percent         |              | Nil                             |              | 0.040                 |              | 0.058                 |
| Yield Finished Oil, Percent    |              | 94.0                            |              | 95.0                  |              | 92.8                  |

lated by temperature control device 14 and thence through pipe 40 to a second condensate settler 41. As in the previous settling stage the condensed steam is removed through the condensate drain 36 while the oil is passed overhead through pipe 42 to a dehydrating device of any conventional type, but shown diagrammatically in the drawing as a flash evaporator 43. A back pressure regulator diagrammatically shown at 44 is interposed in the line 42 and a vacuum is imposed on evaporator 43 through pipe 45. The dry acid treated neutral oil is withdrawn from the evaporator through pipe 46.

For best results the washing stages 24 and 37 are operated above 212° F. at which temperatures the viscosity and surface tension of the oil are lowered facilitating good mixing. It is essential that the settlers 24, 34 and 41 be operated entirely in the liquid phase and in order to prevent vaporization of water under the conditions of temperature which are desirable for good settling it is necessary to hold a back pressure on the system in excess of the vapor pressure of water at the operating temperatures.

The quantity of steam used in the washing steps 24 and 37 may vary between 10 pounds and 150 pounds per barrel of oil per washing stage. Normally the settling time required in both the neutralization settler and the steam condensate settlers will be short but in some instances as much as three hours may be required. Pilot plant operations show that sulfonate bodies, ash and some color-bearing constituents are not completely removed by hot water washing but are definitely removed from the acid treated oil when steam is employed in one or more steam washing stages.

There is shown below a tabulation wherein a comparison is made of the results between a three-stage steam injection washing and two three-

On the graph shown in Fig. 2 are plotted curves showing the effect of water and steam washing. The effect of the water washing operation is indicated in the upper line and the steam washing operation in the lower line. The dotted lines indicate the probable shape of the curves in the unexplored region at very low acid dosages. These curves were developed from the treatment of the same (2200) viscosity SSU Texas distillate described above using 98% sulfuric acid dosages according to the pounds per barrel shown with the resultant NPA colors. This curve clearly shows that it is possible to get a given color with much less acid when utilizing steam washing than when using water washing.

To produce a finished oil having: 4½ NPA color; ash, nil; neutral No. 0.03 or less; carbon residue 0.50 or less, it was found necessary from pilot plant operation, as shown by the schedule, to use 3-stage steam injection washing. The charging stock for each treatment, as indicated in the schedule, while substantially the same, differed slightly in respect to viscosity due to the fact that each of the three samples was taken from a different tank of oil. All requirements of the finished oil specification were met by washing with steam in three stages when using 6 pounds of 98% sulfuric acid per barrel and a 94% yield of product was obtained. To accomplish the same results when using three-stage water washing it was found, as shown in the tabulation, that it was necessary to use 16½ pounds acid per barrel and even then ash specifications were not met. The product yield also fell off to 92.8%. To show the improvement of steaming there has been listed a three-stage water washing operation using only 6 pounds of acid per barrel of oil resulting in 6 NPA color and 0.04 ash which properties do not meet the necessary specifications.

It will be seen from the above that there is a decided improvement and unexpected result obtained by substituting steam washing in place of water washing. Why the improvement occurs is not definitely known but the results in so far as improvement of product, yield and removal of ash and carbon residue speak for themselves.

From the foregoing it will be seen that this invention is one well adapted to attain all of the ends and objects hereinabove set forth together with other advantages which are obvious and which are inherent thereto.

It will be understood that certain features and subcombinations are of utility and may be employed without reference to other features and subcombinations. This is contemplated by and is within the scope of the claims.

As many possible embodiments may be made of the invention without departing from the scope thereof it is to be understood that all matter herein set forth or shown in the accompanying drawings is to be interpreted as illustrative and not in a limiting sense.

Having thus described my invention, I claim:

1. A process of neutralizing and finishing lubricating oil preliminarily treated with acid, comprising the steps of contacting the acid treated oil with a neutralizing agent in amounts sufficient to neutralize the oil and separating the neutralizing agent from the oil, then contacting the oil in a closed system with steam and finally condensing the steam and separating the oil from the condensed steam.

2. A process of neutralizing and finishing lubricating oil preliminarily treated with acid,

comprising the steps of contacting the acid-treated oil with a neutralizing agent in amounts sufficient to neutralize the oil and separating the neutralizing agent from the oil, then contacting the oil with steam in a closed system in a plurality of successive stages and condensing the steam and separating the oil from the condensed steam after each steam contacting stage.

3. A process of neutralizing and finishing lubricating oil preliminarily treated with acid, comprising the steps of contacting the acid-treated oil with a neutralizing agent in amounts sufficient to neutralize the oil and separating the neutralizing agent from the oil, then contacting the oil with steam in a closed system in a plurality of successive stages and cooling the oil after each steam contacting stage to remove moisture condensate and finally separating the remaining moisture from the oil by evaporation.

CHARLES WALCOTT STRATFORD.

#### REFERENCES CITED

The following references are of record in the file of this patent:

#### UNITED STATES PATENTS

| Number    | Name     | Date          |
|-----------|----------|---------------|
| 1,761,328 | Chappell | June 3, 1930  |
| 1,816,872 | Rial     | Aug. 4, 1931  |
| 2,361,455 | Chechot  | Oct. 31, 1944 |

#### OTHER REFERENCES

Koetschau: Z. Angew. Chem., 32, 45-6 (1919), C. A. 13, 2758-9 (1919).